

Sept. 15, 1925.

1,553,907

L. H. MARSHALL

METHOD OF TREATING MALLEABLE CAST IRON AND PRODUCT THEREOF

Filed April 21, 1923



Inventor

LESLIE H. MARSHALL

Witness:-

G. S. Allenbaugh

By

*James*

Attorney

## UNITED STATES PATENT OFFICE.

LESLIE H. MARSHALL, OF MANSFIELD, OHIO, ASSIGNOR TO THE OHIO BRASS COMPANY, OF MANSFIELD, OHIO, A CORPORATION OF NEW JERSEY.

## METHOD OF TREATING MALLEABLE CAST IRON AND PRODUCT THEREOF.

Application filed April 21, 1923. Serial No. 633,789.

To all whom it may concern:

Be it known that I, LESLIE H. MARSHALL, a citizen of the United States of America, residing at Mansfield, in the county of Richland and State of Ohio, have invented certain new and useful Improvements in Methods of Treating Malleable Cast Iron and Products Thereof, of which the following is a specification.

10 This invention relates to metallurgy. More specifically it relates to a process of treating malleable cast iron and to the product of that process.

One of the objects of the invention is to provide a process of treating malleable cast iron whereby certain new and valuable properties are imparted thereto.

Another object is to provide malleable cast iron having new and valuable properties and characteristics.

Other objects are to provide a process of galvanizing, sherardizing, or otherwise coating malleable iron without impairing the properties of the iron and to provide malleable cast iron so coated and having certain new properties and characteristics. Still further objects will appear as the invention is hereinafter disclosed.

For many years it has been found that hot galvanizing, sherardizing, or similarly treating malleable cast iron renders a comparatively large portion of a heat, brittle, less ductile, crystalline in fracture and low in resistance to shock, while the remainder of the same heat possesses its properties and characteristics substantially unimpaired. In the heretofore unsuccessful efforts to solve the problem of galvanizing, sherardizing or similarly coating, malleable cast iron to secure a uniform product of substantially unimpaired characteristics and properties, many different theories have been advanced among which are the following: that the composition of the hard iron before malleableizing affects the ultimate product, that the treatment of the iron in the annealing or malleableizing process enters into the problem, that the process of pickling or cleaning the castings, the temperature of the zinc bath, the temperature of the quenching bath, the rate of cooling after coating, the dissolving action of the

molten zinc, or combinations of these and other steps enter into the problem.

I have discovered that as the temperature of normal malleable cast iron is raised it passes successively through the following ranges or zones of temperature:

(a) A danger zone, i. e., a range of temperature such that if the iron is raised to a temperature within that zone and subsequently cooled, the iron often, though not invariably, becomes brittle and otherwise changes its properties.

(b) A neutral point, i. e. a temperature at which the iron, when raised to that temperature and then cooled, possesses substantially the same degree of malleability or resilience as it possessed before heating, and

(c) A safety zone, i. e., a range of temperature such that if the iron is raised to a temperature within that zone and subsequently cooled, the malleability and other desirable properties of the iron will be maintained or improved.

My heat treating process differs from the annealing or re-annealing processes of the prior art in various respects among which are the following: When the so called "hard iron" is annealed to produce malleable properties therein or the annealed iron re-annealed, it is brought to a temperature above that of the carbon-combining or critical temperature of that particular iron, maintained at that temperature for a period depending upon the composition of the iron and the temperature to which it has been raised, and subsequently cooled. In my process of treating malleableized iron, the temperature of the iron is not raised above the carbon-combining or critical temperature, but its maximum temperature is kept below the critical temperature. Again, malleable cast iron which has been annealed or re-annealed, in accordance with the processes of the prior art, is not stable but when subsequently raised to a temperature within the danger zone (as in case of hot galvanizing or similarly coating) is beyond control of the operator in that he has no assurance that the iron will not become embrittled, and large quantities of malleable iron castings commonly become embrittled whereas others

are reliable, though the composition and annealing process are apparently the same in either case. On the other hand, the product of my process is stable, i. e., it uniformly retains its malleability even when subsequently heated to a temperature within the danger zone as in hot galvanizing or similarly coating the iron.

Explanation of my discovery and novel process may be facilitated by reference to the drawing which indicates graphically the results of actual tests made by me. The curves A and B are plotted with temperature in degrees Fahrenheit as abscissa and impact values in percentage of original impact value as ordinates. Curve A represents graphically the result of certain tests and observations made in connection with different specimens all from the same piece of commercial normal malleable cast iron. In making these tests I heated different specimens from 392° F. to a corresponding one of a number of different temperatures between 392° F. and 1472° F., held each particular specimen at its higher temperature for three minutes and then quenched in water at 175° F. After quenching, each specimen was tested in an impact machine of the Izod type to determine its resiliency. Such use of an Izod machine is known to those skilled in the art. It consists in measuring the foot pounds required to fracture a notched specimen (notching is standard practice) under test. As to each specimen, I plotted the temperature to which it had been raised as the abscissa and the percentage impact value of that specimen, as determined from the Izod test machine, as the corresponding ordinate. Therefore, the ordinate of each point on the curve A represents to scale, on a basis of 100 as the impact value of normal malleable cast iron before heating, the percentage impact value of a particular one of a number of specimens, all taken from the same piece of commercial malleable cast iron, and which particular specimen has been raised to a temperature indicated by the corresponding abscissa, and then subsequently treated by quenching as above described.

It will be observed that as the treating temperature is increased from 392° F. to substantially 700° F. the resulting malleable cast iron shows increasing embrittlement to a point where the resistance to breaking is only about 16% of that of the untreated product. From 700° F. to 1020° F. the effect of increasing the temperature does not appear to further increase the embrittlement, but at approximately 1020° F. the curve suddenly rises, crossing the 100% line which I have termed the normal line, at a temperature of 1103° F., and reaching a point where at a temperature of 1130° F.

the resistance under impact to breaking is approximately 154% of the untreated product, thus indicating that if the normal or commercial malleable cast iron represented by curve A is subjected to a heat treatment of approximately 1130° F., and then quenched, the impact value is raised above that of the untreated iron, or to be exact, the product will withstand a 54% greater impact blow than the untreated product before it will break and is therefore more resilient. By increasing the temperature above 1130° F. and up to substantially 1400° F. (the critical temperature at which the free carbon in this iron begins to recombine) the resistance to impact is lowered slightly from that at 1130° F., and the curve further shows by its sudden drop that a heat treatment above 1400° F. will cause a decrease in the resiliency as shown by the decrease in the impact value.

The malleable cast iron upon which the tests shown by curve A in Fig. 1 are based, contained

|              |        |    |
|--------------|--------|----|
| Total carbon | 2.10 % | 90 |
| Silicon      | .80 %  |    |
| Phosphorus   | .20 %  |    |
| Manganese    | .26 %  |    |
| Sulphur      | .073%  |    |

Inspection of curve A will indicate that the danger zone of the particular malleable cast iron there graphically shown lies below 1103° F. and that the safety zone thereof lies between 1103° F. and 1400° F. The neutral point or temperature marks the dividing point between the danger and safety zones and this neutral point is indicated by the intersection of the curve with the 100% line, the abscissa of the intersection being 1103° F. It will be noted that the curve A is quite steep at its intersection with the 100% line and rises rapidly to a peak at about 1130° F. In other words, if the particular iron is raised to a temperature of about 1103° F. and then quenched its impact value will be the same as when untreated but when raised to a temperature of about 1130° F. and then quenched the impact value is increased substantially 54%. In view of these facts and the difficulty of close temperature control or regulation, it is preferable to raise the temperature of the iron to at least 1130° F., and better still 1200° F., and then quench to insure that the impact value of the product shall be no less than 100%, and to secure an otherwise desirable product.

In curve B, Fig. 1, I have shown the results of tests upon a grade of malleable cast iron containing 3.15% of carbon, .63% of silicon, phosphorus .15%, manganese .31% and sulphur .08%. The specimens were subjected to the same treatment as the specimens

covered by curve A. Curve B differs from curve A as would be expected on account of the difference in the chemical composition, but here too we find a zone of heat treatment which will produce embrittlement and a zone of heat treatment which will improve the resiliency or impact value of the iron over and above that of the untreated iron. The iron represented by curve B shows that it is not necessary to heat it to the temperature required by the iron represented by curve A and the increase in impact value is not as great, neither is the embrittlement as great when heated within the danger zone. This iron is not as sensitive to a temperature below the neutral point and does not respond in as great a degree in increased resiliency with the heat treatment, as the iron covered by curve A, but still curve B shows that, as in the case of curve A, there is a distinct embrittlement zone, and a distinct temperature zone within which the iron can be treated and improved.

I have further found that normal or commercial malleable cast iron having a composition of total carbon 2.35%, silicon .91%, phosphorus .18%, manganese .25% and sulphur .051% when heat treated to a temperature of approximately 1200° F. and then quenched in water at 175° F., that the impact value as measured by the Izod type of impact machine was 148% of the impact value of the same malleable cast iron untreated or 48% greater.

Tests thus far made by me indicate that the time rate of temperature increase in bringing the iron up to the treatment temperature is of relatively minor importance.

Limited tests made to date seem to indicate that the rate of cooling from the heat treatment temperature has some effect upon the impact value or resiliency of the heat treated iron, in that quenching in the air tends to give a product of a higher impact value than quenching in hot water or oil and when allowed to cool with the heating furnace an even higher impact value is secured as shown by the following table which shows the results secured upon the same malleable cast iron used in the tests represented by the curve A in Fig. 1.

| Time at 1255° F.         | Method of quenching.     | Impact value. |
|--------------------------|--------------------------|---------------|
| 3 minutes.....           | Cooled with furnace..... | 181           |
| 3 minutes.....           | In air.....              | 140           |
| 3 minutes.....           | In hot water 175° F..... | 133           |
| Same iron untreated..... |                          | 100           |

Likewise experiments seem to indicate that the length of time that the malleable cast iron is maintained or held at the heat treating temperature has an influence upon the resilient properties thereof, as shown by the following table compiled from tests and

observations of the same iron as was tested to obtain the immediately preceding table.

| Time at 1200° F.         | Quenched.            | Impact value. | 70 |
|--------------------------|----------------------|---------------|----|
| 300 minutes.....         | In water—175° F..... | 128           |    |
| 50 minutes.....          | In water—175° F..... | 156           |    |
| 3 minutes.....           | In water—175° F..... | 133           |    |
| Same iron untreated..... |                      | 100           |    |

Bearing in mind that hot galvanizing of malleable cast iron is accomplished in a zinc bath at a temperature not less than the melting point of the zinc employed (approximately 787° F.) and not to exceed approximately 900° F., it will now be appreciated, in view of my discovery above set forth, that such hot galvanizing is carried on well within the danger zone of the malleable cast iron (see curves A and B), i. e., the zone of temperature at which the worst embrittlement commonly occurs. And this fact is borne out by experience in the practical art of hot galvanizing malleable iron castings.

A further and very important feature of my discovery and invention resides in the fact that after malleableized cast iron is heated to cause its temperature to pass through and beyond the danger zone and into the safety zone and then further treated as above described by quenching, it retains the resiliency or impact value and other desirable characteristics and properties imparted to it by such treatment even when subsequently heated to carry it into the danger zone and on the danger zone side of the neutral point or temperature. Thus I found, after treating specimens of malleable cast iron as set forth in connection with curves A and B (including the step of elevating the temperature of the iron into the safety zone) and subsequently reheating the iron to 844° and quenching in water at 175° F., that the reheating after the heat treatment did not decrease the impact value. In other words the benefits secured by the heat treatment at 1200° F., or other temperature within the safety zone including the steps of quenching, remain fixed. In fact, after heat treatment to 1200° F. and subsequent reheating to 844° F., malleable cast iron showing an impact value of 160% of the untreated iron has been produced by me. The same heat treatment and reheating just described, when carried out on normal malleable cast iron having a carbon content of 2.10% and a silicon content of 0.80% showed an impact value of 139% of the impact value of specimens before treatment in accordance with my process.

I have also found that my process is not only effective in preventing the embrittlement of commercial malleable cast iron, but that the iron represented in curve A if it has become embrittled, as by hot galvaniz-

ing, sherardizing, etc., may be reclaimed by heat treating such embrittled product between the limits of 1130° F. and 1400° F. (limits approximate) and permitting it to 5 remain at such temperature for a time and then quenching slowly or rapidly depending upon the results desired as disclosed above. Such heat treatment of the embrittled iron will not only restore its resiliency to the same or a greater degree than it originally possessed, but permit it to be again hot, galvanized, sherardized, etc., without endangering its malleable properties.

Recapitulating—in accordance with my 15 invention, I have provided a process of treating normal malleable cast iron whereby its malleability and other desirable properties possessed by it prior to treatment are maintained, or preferably increased, and 20 retained even though subsequently heated to a temperature within and not beyond the danger zone; a novel product, i. e., malleable cast iron having high resilience and other desirable characteristics and properties 25 and which are retained though the iron be heated to a temperature within and not beyond the danger zone; a process of hot galvanizing or similarly coating malleable cast iron without impairing, but if desirable 30 increasing, its resilience and other desirable properties; novel galvanized or similarly coated malleable cast iron products; and a process for reclaiming malleable cast iron which has been embrittled by hot galvanizing 35 or otherwise coating it in accordance with the processes of the prior art. It is my present intention to direct the claims of the present application to the process of treating malleable cast iron which as above 40 described includes the steps of heating the iron to a temperature within the safety zone, maintaining it at such temperature for the desired length of time, and then cooling the iron by quenching; and to claim the other 45 features of invention, herein disclosed, in one or more divisional or continuing applications.

The embrittlement is shown, by my investigations, to be overcome when normal 50 malleable cast iron is subjected to the process herein disclosed, and actual practice in the application of my process has proved conclusively that my process is practical and can be applied without expensive equipment, 55 and where the loss due to hot galvanizing, embrittling the iron has been very large and uncontrollable, such loss will be practically eliminated by my invention.

The process described can be carried out 60 by placing the commercial malleable cast iron castings to be heat treated in a furnace having a source of heat to bring them up to the temperature required preferably within the safety zone, and allowing them to remain 65 at the desired temperature for a period of

time and sufficient to insure that the temperature is uniform throughout the material treated which may be found to give the best results and then quenched by cooling within the furnace, or removed from the furnace and 70 quenched in air, water, etc., as may be found to give the desired results, or a continuous type of furnace may be used and the castings run out and quenched in air, water or oil at such temperature as desired, and the process 75 made continuous or other means of securing the desired temperature may be used.

I have found that my process is applicable to malleable cast iron of varying chemical composition, and which has been put through 80 the recognized commercial annealing treatment in the malleableizing process. In this case, the novel treatment may be applied to the iron by quenching it after its temperature has been brought below the critical or 85 carbon-combining temperature and before its temperature has dropped below the safety zone of temperature described above.

In view of the variable conditions met with in commercial malleable cast iron I do 90 not wish to be limited strictly to any specific temperature, time, rate of cooling or other conditions, as different grades or compositions of iron may change the temperature treatments required, as already shown by 95 curves A and B, and some grades of iron may require different times under the treatment temperature and different rates and means of cooling, nor do I wish to be limited to the composition of the malleable cast iron 100 to which my invention is applicable. I have found, however, that there is a definite range of temperature, for a given grade of malleable cast iron, between the limits of which the iron is embrittled and another range, between the limits of which the iron is improved (see Fig. 1) and rendered immune 105 from embrittlement when again heated at a lower temperature as in galvanizing.

I find that treating at a temperature of 110 approximately 1200° F., and then quenching will as a rule secure the desired results, as this temperature falls safely within the heat treatment or safety zone of most grades of 115 commercial malleable cast iron.

From the curves shown in Fig. 1 it will be apparent to one skilled in the art that since there are two well defined zones as described, and that heating normal malleable cast iron to a temperature within the zone which I have specified, as the safety zone 120 and then quenching will protect the iron from embrittlement when reheated to a temperature falling within the danger zone, that one who is producing malleable cast iron 125 or one who is using malleable cast iron can stabilize or protect the same against embrittlement by subjecting the iron to a series of tests at different temperatures to determine exactly the limits of the "safety" and "dan-

ger" zones, or by determining the limits of the "safety" zone of the particular iron and heat treating the iron according to the results determined and the method I have disclosed.

- 5 To hot galvanize malleable cast iron castings I first subject them to a temperature within the range of the heat treating or safety zone as described and then cool or quench as described, and then subject them to the 70  
10 regular hot galvanizing process which consists in cleaning the castings and placing them in the hot zinc bath and then quenching in air, hot water or oil, which process requires no extended description herein.
- 15 As stated above, my process of hot galvanizing or otherwise coating malleable iron and the new products are not claimed herein.

In the appended claims I use the word 20 quenched, or quenching, to indicate air cooling; or liquid cooling; or cooling in a furnace but at a comparatively rapid rate such, for example, as would take place in a comparatively small or experimental furnace as 25 distinguished from a large commercial furnace.

What I claim is:—

1. The process of treating malleableized cast iron comprising heating the iron in a 30 continuous furnace to a temperature within the safety zone, and then quenching the iron.
2. The process of treating malleableized cast iron consisting in heating the iron to approximately 1200° F., and then quenching.
- 35 3. The process of treating malleableized cast iron comprising placing the iron in a furnace and bringing the iron to a temperature of approximately 1200° F., and holding the iron at this temperature and then quenching the iron to immunize the iron against danger of embrittlement when reheated below its neutral temperature.
4. The process of treating malleableized cast iron comprising heating it to a temperature not to exceed its critical temperature and then quenching, whereby the iron is rendered immune from embrittlement when/if later heated below its neutral temperature.
- 50 5. The process of treating malleableized cast iron comprising heating the iron to a temperature not to exceed its critical temperature and whereby it is rendered immune from embrittlement when/if later heated below the neutral temperature.
- 55 6. The method of treating malleableized cast iron which comprises heating the iron to cause its temperature to rise through the zone of temperature at which the iron is in danger of embrittlement, and cooling the iron before the carbon-combining temperature is reached.
- 60 7. The process of treating malleableized cast iron comprising heating the iron to a temperature not to exceed substantially

1400° F. and not below a temperature which will tend to decrease the impact value of the iron below that of the untreated iron.

8. The process of treating malleableized cast iron consisting in heating the iron to a 70 temperature not to exceed substantially 1400° F. and not below a temperature which will tend to decrease the impact value of the iron below that of the untreated iron and then quenching the iron.

9. The method of treating malleableized cast iron which has a thermal zone between the limits of which the iron is embrittled if heated and another thermal zone between the limits of which the iron is rendered immune from embrittlement if heated, said method comprising heating said iron to a temperature falling within the limits of said latter zone.

10. The method of treating malleableized cast iron which has a thermal zone between the limits of which the iron is embrittled if heated and a thermal zone between the limits of which the resiliency of the iron is increased over and above that of the untreated 90 iron, said method comprising heating the iron to a temperature falling within the limits of said latter zone, and then quenching the iron.

11. The method of treating malleableized cast iron which has a thermal zone between the limits of which the iron is embrittled if heated and another thermal zone between the limits of which the iron is rendered immune from embrittlement if heated, said method consisting in heating said iron to a temperature falling within the limits of said latter zone and then quenching the iron.

12. The method of producing malleable cast iron comprising the steps of annealing the iron in the hard iron condition to change the combined carbon into free or graphite carbon, then stabilizing the annealed iron by heating it to a temperature in excess of that which will cause the iron to be embrittled, and then quenching the iron.

13. The method of heat treating malleable cast iron comprising first subjecting a plurality of like samples of the iron each to a different temperature between room temperature and its critical temperature for a uniform period of time, then uniformly cooling, and then subjecting each sample to a mechanical test which will measure its resiliency, then comparing the results with a like test upon a like sample untreated and then subjecting the iron to be treated to a temperature in excess of that which it is found by the samples treated to give a greater degree of resiliency than the untreated sample.

14. The method of reclaiming malleable cast iron which has been embrittled by heating to below the neutral temperature, comprising heating the iron to a temperature

75

80

85

95

100

105

110

115

120

125

130

between the neutral temperature and the critical temperature.

15. The method of reclaiming malleable cast iron which has been embrittled by heating to a temperature below the neutral temperature, comprising heating the iron to such temperature below the critical temperature as will remove said embrittlement.

16. The method of heat treating malleableized cast iron comprising subjecting the iron to a temperature in excess of its neutral temperature and below its critical temperature.

17. The method of producing malleable cast iron comprising the step of heating the iron to a temperature above the carbon-combining temperature, maintaining the iron at that temperature for a period dependent upon the composition of the iron and the temperature to which it has been raised, and cooling the iron to a temperature below the carbon-combining temperature, in accordance with the ordinary American commercial annealing operation; and then quenching the iron while its temperature is above the neutral temperature.

18. The method of improving the physical properties of malleableized cast iron comprising heat treating the iron to a temperature falling within the safety zone described, and then quenching the iron.

19. The method of treating malleableized cast iron comprising in first subjecting the iron to a test to determine the neutral temperature and then heating to a temperature

above the neutral temperature and below the critical temperature.

20. The method of stabilizing the malleability of malleableized cast iron which comprises heating the iron to cause its temperature to pass through the zone of temperature at which the iron is in danger of becoming embrittled, and cooling the iron before the carbon-combining temperature has been reached.

21. The process of improving physical properties of normal malleableized cast iron consisting in heat treating the iron to a temperature within the saftey zone and then quenching.

22. The method of producing malleable cast iron comprising the steps of heating the iron to a temperature above the carbon-combining temperature, bringing the iron to a temperature below the carbon-combining temperature, and then quenching the iron while its temperature is above that which will cause the iron to be in danger of embrittlement.

23. The method of producing malleable cast iron comprising the steps of heating the iron to a temperature above the carbon-combining temperature, bringing the iron to a temperature below the carbon-combining temperature, and then quenching the iron in liquid while its temperature is above that which will cause the iron to be in danger of embrittlement.

In testimony whereof I affix my signature.  
LESLIE H. MARSHALL.